

H. F. FRENCH,  
PROCESS OF MAKING BATTERY ANODES,  
APPLICATION FILED DEC. 27, 1915.

1,359,244.

Patented Nov. 16, 1920.

Fig. 1



Fig. 2



Fig. 3



INVENTOR.  
HARRY F. FRENCH  
BY *Ira J. Adams*  
ATTORNEY

# UNITED STATES PATENT OFFICE.

HARRY F. FRENCH, OF FREMONT, OHIO, ASSIGNOR, BY MESNE ASSIGNMENTS, TO NATIONAL CARBON COMPANY, INC., A CORPORATION OF NEW YORK.

## PROCESS OF MAKING BATTERY-ANODES.

1,359,244.

Specification of Letters Patent. Patented Nov. 16, 1920.

Application filed December 27, 1915. Serial No. 68,605.

To all whom it may concern:

Be it known that I, HARRY F. FRENCH, a citizen of the United States, residing at Fremont, in the county of Sandusky and State 5 of Ohio, have invented a certain new and useful Improvement in Processes of Making Battery-Anodes, of which the following is a full, clear, and exact description.

My invention relates to electric batteries 10 employing zinc as the positive electrode, and while not necessarily restricted thereto, the invention is particularly applicable to batteries with alkaline electrolyte.

It has been the practice in the past to 15 construct primary alkaline batteries with copper oxid depolarizer, with either rolled or cast zinc as the positive electrode. Cast zinc seems to have some advantages over rolled zinc, which is probably due to its 20 crystalline structure, but I have found that both are inferior to specially cast zinc, which is the subject of this invention.

Zinc electrodes as ordinarily cast are 25 cooled quickly by the relatively cold mold and have small crystals arranged in such a way that they all point inward from the sides and edges. This structure of the zinc may be plainly seen by breaking a zinc casting.

30 I have found that if the zinc casting is cooled slowly it changes its structure entirely and consists of large crystals arranged in such a way that its fracture has the appearance of superposed layers or flakes of zinc particles extending across the plate.

When a zinc casting, as ordinarily cast, is subjected to sufficient stress to break it, it breaks very suddenly, as it is quite brittle. However, with the slowly cooled zinc casting, the zinc is not brittle, but will bend 40 considerably without breaking, when subjected to sufficient bending stress. Also the bending of the specially cast zinc produces a "cry" resembling the noise emitted by a 45 rod of lead or solder when bent suddenly.

Referring to the drawing, in which like numerals of reference designate similar parts throughout, Figure 1 is a plan view of the filled mold. Fig. 2 is a side view 50 showing heating means applied to the mold

and Fig. 3 is an elevation of the device shown in Fig. 1.

I am not able to specify exact time-temperature gradients in casting the new zinc electrode, but I have found the following 55 process to produce the desired product. A 5-inch by 7-inch by  $\frac{7}{8}$ -inch rolled zinc plate 1 is placed on an iron plate 2 about 9 inches long, 7 inches wide and  $\frac{1}{4}$  inch thick. Iron strips 3, 4, 5 and 6 about  $\frac{3}{4}$  inch square 60 in cross section, are placed around the edges of the zinc to serve as sides of the mold.

Heat is next applied by any appropriate means, conveniently one or more gas burners 7, as shown, until the zinc melts. The 65 source of heat is then shut off and the zinc allowed to cool down and solidify. I have also found that cooling can be hastened somewhat by directing an air blast on the zinc after it has solidified, without detriment. Here again, I have no data to give in regard to the rate of cooling but I direct an air blast on the bottom of the iron plate of the mold, from a  $\frac{3}{8}$  inch gas cock in a pipe or hose containing air at 20 pounds gage 70 pressure. This can be directed on the plate as soon as the heat is turned off, without detrimental effect.

Instead of melting rolled zinc in a mold, as given above by way of example, I may 80 also melt ordinary cast zinc or zinc ingots, or hot molten zinc, may be poured into the heated mold and allowed to cool, as the essence of the invention is in the relatively slow cooling of the zinc. In ordinary die-casting, the mold heats up to some extent on account of the heat absorbed from the zinc, but it is relatively cool as compared with the heated mold in this invention; since such mold is heated up to the melting point 85 of zinc. It is not necessary to have the mold heated exactly to the temperature of molten zinc in case molten zinc is poured into it; but it must be heated much higher than the temperature of the mold in ordinary zinc casting.

When electrodes are made of the zinc cast in accordance with the preceding process, the zinc and its impurities function somewhat differently when used in a battery, so 100

that much less mercury is required to amalgamate the electrodes. I have found that in most cases only about  $\frac{1}{5}$  the usual amount of mercury is necessary to properly amalgamate the new form of zinc electrodes, as determined by their performance in the battery cell.

With the new zinc electrodes, impurities, such as lead and cadmium, are much less liable to scale or flake off and short circuit the cell, or to coat over with incrustations as do ordinary rolled or cast zincs. Both of these characteristics materially increase the life of the cell by permitting more of the

zinc to be dissolved and by keeping the voltage up for a longer time than would be the case if the regular form of zinc were used.

Having described my invention, what I claim is:—

The process of making a zinc battery electrode which consists in forming it into shape in a mold heated to substantially the melting temperature of zinc, and cooling the mold so that the zinc is solidified slowly.

In testimony whereof, I hereunto affix my signature.

HARRY F. FRENCH.